

2,881,139

## CORROSION PREVENTING COMPOSITIONS AND PROCESS

Hermann Gysling, Basel, Switzerland, assignor to J. R. Geigy A.-G., Basel, Switzerland, a Swiss firm

No Drawing. Application August 22, 1955  
Serial No. 529,913

Claims priority, application Switzerland  
September 16, 1954

15 Claims. (Cl. 252—137)

The present invention concerns a process for the protection of copper and copper alloys with base metals against corrosion when in contact with water or aqueous alkaline solutions. It also concerns agents, in particular cleansing agents, the aqueous or aqueous-alkaline solutions of which, due to a content of the protective agents against corrosion usable according to the present invention, have no or only an inconsiderable corrosive action on scoured surfaces of copper and alloys thereof with base metals.

It has been found that scoured surfaces of copper and alloys of copper and base metals can be protected against corrosion in contact with water and in particular with aqueous alkaline solutions if slight amounts of such 2-guanidino-aryloimidazole compounds containing no water solubilising groups which dissociate acid in neutral water and which are at least very slightly soluble in water or in aqueous solutions, are added to the water or to the solutions.

2-guanidino-aryloimidazole compounds used according to the present invention can contain as aryl radicals, for example, the benzene or the naphthalene ring which can be further substituted, for example with halogen, alkyl, alkoxy, nitro, acylamino, alkylsulphonyl, arylsulphonyl or sulphonic acid amide groups. They may not contain, however, any groups either as such or in the form of their water solubilising salts which dissociate acid in neutral water such as, for example, carboxyl, sulphonic acid or phosphonic acid groups. As they must be water soluble, even if only slightly so, the benzimidazole compounds are to be preferred to those with higher condensed rings. For example, 2-guanidino-benzimidazole, 2-guanidino-6-chloro-, -6-methyl-, -6-methoxy- or -6-ethoxy-benzimidazole, 2-guanidino-4- or -6-nitro-benzimidazole, 2-guanidino-4- or -6-acylamino-benzimidazole, 2-guanidino-6-methylsulphonyl-, -ethylsulphonyl-, or -n-butylsulphonyl-benzimidazole, 2-guanidino-benzimidazole-6-sulphonic acid dimethylamide, -diethylamide, -piperide or -morpholide, 2-guanidino-4.5:1'2'-naphthimidazole can be used. Because of its easy accessibility and favourable water solubility, 2-guanidino-benzimidazole is to be preferred to all other compounds.

Some of the 2-guanidino-aryloimidazole compounds useable according to the present invention are known but all can be produced easily according to known methods from aromatic o-diamino compounds by condensation with dicyanodiamide in acid solution.

Very small amounts of these 2-guanidino-arylo-imidazole compounds, for example 0.1 to 100 mg. per litre, protect scoured copper and alloys thereof with base metals such as, e.g. brass or nickel silver, from corrosive action when in contact with water or aqueous alkaline solutions, in particular in a pH range of from 8 to 12. The aqueous alkaline solutions can contain for example lithium, sodium or potassium salts of carbonic acid or the oxy acids of boron, silicium or phosphorus having a basic reaction. They may also contain neutral salts such

as sodium sulphate, sodium chloride, potassium sulphate or potassium chloride etc. such as are the usual additives to capillary active cleansing agents as well as capillary active wetting, dispersing and cleansing agents which contain lipophilic hydrocarbon radicals and hydrophilic groups. Examples of such capillary active agents are: the fatty alcohol polyglycol ethers, the alkyl phenol polyglycol ethers, the fatty acid alkanol amides and polyglycol ethers thereof, the alkali and ammonium salts of the sulphuric acid half esters of fatty alcohols, of the sulphated mono-fatty acid esters of polyalcohols, the alkali and ammonium salts of alkyl and alkylaryl sulphonate acids, of sulphosuccinic acid esters and of fatty acids which contain lipophilic radicals.

Particularly in aqueous-alkaline solutions of wetting, dispersing and cleansing agents which contain the usual alkali salts of polyphosphoric acids which make calcium ions unharful, such as e.g. tetrasodium pyrophosphate, pentasodium triphosphate, sodium hexametaphosphate or mixtures of the alkali salts of such polyphosphoric acids, the 2-guanidino-arylo-imidazole compounds used according to the present invention protect scoured copper and alloys thereof with base metals from corrosion when in contact with these solutions. They also protect copper from attack by aqueous ammonia and amines. It is of advantage therefore, to incorporate them in alkaline cleansing agents made up from salts having an alkaline reaction such as alkali carbonates, alkali silicates, alkali borates and alkali polyphosphates or in cleansing agents which contain such salts as well as, possibly, capillary active wetting and cleansing agents and neutral salts which are used for the treatment of scoured copper and alloys thereof with base metals. The content of corrosion protective agents according to the present invention depends to a great extent on the specific activity of the 2-guanidino-aryloimidazole compound used, on the alkalinity of the treatment liquor, and on the temperature and duration of the treatment. Generally amounts of up to 1% calculated on the non-aqueous components of such cleansing compositions are sufficient but also considerably less or more can be incorporated, for example 0.05 to 5%.

The following examples illustrate the invention without limiting it in any way. Where not otherwise stated, parts are given as parts by weight and the temperatures are in degrees centigrade.

### Example 1

An aqueous solution containing

4.0 g. tech. tetrasodium pyrophosphate  
1.0 g. 2,4-di-tert. amylphenol polyglycol ether

per litre attacks brass plate and nickel silver plate while forming strong oxidation tints; in addition some of the metal dissolves. At a temperature of 55 to 60° over a period of 24 hours, the loss in weight of elementary metal is

Brass ----- 7.0 g./sq. m./24 hours  
Nickel silver ----- 14.6 g./sq. m./24 hours

If 3 mg. of 2-guanidinobenzimidazole is added for every litre of the above treatment liquor and a parallel test is made then, under the same conditions, there are the following losses in weight:

Brass ----- 0.25 g./sq. m./24 hours  
Nickel silver ----- 0.46 g./sq. m./24 hours

This shows that by the addition of a protective agent, the corrosion can be reduced to a fraction of what it would otherwise have been. In addition, in this test the scoured shining appearance of the untreated platings is retained.

## Example 2

Brass plate and nickel silver plate are treated with 8 g. of the following composition of washing agents in a litre of tap water:

3.0 parts of tetrasodium pyrophosphate,  
1.0 part of the sodium salt of ethylenediamine tetraacetic acid,  
2.0 parts of soap (sodium salt of stearic acid),  
0.5 part of the sodium salt of a secondary alkyl sulphate (Shell's "Teepol").

Both at room temperature and at higher temperatures the platings are corroded and there is strong discolouration. On the other hand, if 0.5 to 5 mg. per litre of one of the 2-guanidinobenzimidazoles listed below are added to the washing liquor then practically complete protection against corrosion is attained: 2-guanidinobenzimidazole, 6-chloro-2-guanidinobenzimidazole, 6-methyl-2-guanidinobenzimidazole, 6-nitro-2-guanidinobenzimidazole, 6-acetylaminoo-2-guanidinobenzimidazole, 6-methoxy-2-guanidinobenzimidazole, 6-ethoxy-2-guanidinobenzimidazole, 6-methyl sulphonyl-2-guanidinobenzimidazole, 6-ethyl sulphonyl-2-guanidinobenzimidazole, 6-butyl sulphonyl-2-guanidinobenzimidazole.

## Example 3

Washing is done in a scoured copper vessel with a composition of washing agents made up as follows:

10 parts of a usual marketed pentasodium triphosphate, 30  
15 parts of tetrasodium pyrophosphate,  
5 parts of sodium silicate (waterglass),  
15 parts of sodium carbonate,  
5 parts of alkylaryl sulphonate (consisting chiefly of dodecyl benzene sulphonate),  
15 parts of fatty alcohol sulphate (lauroyl-sulphuric acid ester),  
1.5 parts of carboxymethyl cellulose,  
0.2 part of an optical brightening agent of the 1,4-bis-triazinylaminostilbene-2,2'-disulphonic acid class,  
33.3 parts of sodium sulphate cryst.

After washing 30 times at 80-90° for 30 minutes each time, the loss in weight of the vessel was 0.50 g. elementary copper for each square metre. In a parallel trial the composition of washing agents was implemented by the addition of 0.05 part (calculated on the solid substances) of 2-guanidinobenzimidazole and the same procedure was followed. In this case, the loss of metal was only 0.06 g. for each square metre. In addition the surface of the copper remained completely scoured.

The other 2-guanidinobenzimidazole compounds listed in Example 2 can be used in this test with the same result.

## Example 4

On contact with scoured copper of a washing liquor containing 8 g. per litre of a composition of washing agents made up from

6 parts of sodium carbonate,  
2 parts of higher fatty acids,  
0.1 part of carboxymethyl cellulose,  
0.8 part of sodium borate,

a strongly coloured oxide layer is formed on the metal even at room temperature and particularly at higher temperatures. If, however, a few milligrammes per litre of one of the inhibitors listed below is added to this washing liquor, then the copper remains completely scoured:

2-guanidinobenzimidazole, 6-chloro-2-guanidinobenzimidazole, 6-methyl-2-guanidinobenzimidazole, 6-ethyl-2-guanidinobenzimidazole, 6-nitro-2-guanidinobenzimidazole, 6-acetylaminoo-2-guanidinobenzimidazole, 6-methoxy-2-guanidinobenzimidazole, 6-ethoxy-2-guanidinobenzimidazole, 6-methyl sulphonyl-2-guanidinobenzimidazole, 6-ethyl sulphonyl-2-guanidinobenzimidazole, 6-

butyl sulphonyl-2-guanidinobenzimidazole, 2-guanidino-4.5:1'2'-naphthimidazole, 2-guanidino-5'-chloro-4.5:1'2'-naphthimidazole.

What I claim is:

5 1. A process of preventing the corrosion of coppery metal surfaces by alkaline aqueous solutions, which comprises bringing said coppery metal surfaces into contact with alkaline aqueous solutions containing from 1 to 100 parts per million of a corrosion inhibitor of the formula



15 wherein Ar represents a member selected from the group consisting of o-phenylene and o-naphthylene radicals which contain no water-solubilizing groups which dissociate acid in neutral water.

20 2. A process of preventing the corrosion of coppery metal surfaces by alkaline aqueous solutions of a water-soluble cleansing agent normally tending in aqueous solution to cause corrosion of coppery metal, which comprises bringing said coppery metal surfaces into contact with alkaline aqueous solutions of a water-soluble cleansing agent containing from 1 to 100 parts per million of a corrosion inhibitor of the formula



wherein Ar represents a member selected from the group consisting of o-phenylene and o-naphthylene radicals which contain no water-solubilizing groups which dissociate acid in neutral water.

35 3. A process of preventing the corrosion of coppery metal surfaces by alkaline aqueous solutions of a water-soluble cleansing agent containing a surface-active agent and alkali metal phosphates, which comprises bringing said coppery metal surfaces into contact with alkaline aqueous solutions of a water-soluble cleansing agent containing a surface-active agent, alkali metal phosphates and from 1 to 100 parts per million of a corrosion inhibitor of the formula



50 wherein Ar represents a member selected from the group consisting of o-phenylene and o-naphthylene radicals which contain no water-solubilizing groups which dissociate acid in neutral water.

55 4. A process according to claim 1, in which the corrosion inhibitor is 2-guanidino-benzimidazole.

5. A process according to claim 1, in which the corrosion inhibitor is 6-nitro-2-guanidino-benzimidazole.

6. A process according to claim 1, in which the corrosion inhibitor is 6-methoxy-2-guanidino-benzimidazole.

7. A process according to claim 1, in which the corrosion inhibitor is 6-methyl-2-guanidino-benzimidazole.

60 8. A process according to claim 1, in which the corrosion inhibitor is 6-chloro-2-guanidino-benzimidazole.

9. A corrosion preventing composition consisting of a water-soluble cleansing agent dissolving in water with an alkaline reaction, the aqueous solutions of which tend to cause corrosion of coppery metal on contact, and of 0.05 to 1%, calculated on the dry weight of said cleansing agent, of a corrosion inhibitor of the formula



wherein Ar represents a member selected from the group consisting of o-phenylene and o-naphthylene radicals which contain no water-solubilizing groups which dissociate acid in neutral water.

10. A corrosion preventing composition consisting of a water-soluble cleansing agent, which comprises a surface-active agent and alkali metal phosphates and which dissolves in water with an alkaline reaction, the aqueous solutions of which tend to cause corrosion of coppery metal on contact, and of 0.05 to 1%, calculated on the dry weight of said cleansing agent, of a corrosion inhibitor of the formula



wherein Ar represents a member selected from the group consisting of o-phenylene and o-naphthylene radicals which contain no water-solubilizing groups which dissociate acid in neutral water.

11. A corrosion preventing composition according to claim 9, wherein the corrosion inhibitor is 2-guanidino-benzimidazole.

12. A corrosion preventing composition according to claim 9, wherein the corrosion inhibitor is 6-nitro-2-guanidino-benzimidazole.

5 13. A corrosion preventing composition according to  
claim 9, wherein the corrosion inhibitor is 6-methoxy-2-  
guanidino-benzimidazole.

14. A corrosion preventing composition according to claim 9, wherein the corrosion inhibitor is 6-methyl-2-guanidino-benzimidazole.

10 15. A corrosion preventing composition according to claim 9, wherein the corrosion inhibitor is 6-chloro-2-guanidino-benzimidazole.

**References Cited in the file of this patent**

UNITED STATES PATENTS

- |           |            |       |               |
|-----------|------------|-------|---------------|
| 2,618,603 | Schaeffer  | ----- | Nov. 18, 1952 |
| 2,618,606 | Schaeffer  | ----- | Nov. 18, 1952 |
| 2,706,179 | Tundermann | ----- | Apr. 12, 1955 |